

## UNITED STATES PATENT OFFICE

KENNETH B. STUART, OF PUEBLO, COLORADO, ASSIGNOR TO THE COLORADO FUEL AND IRON COMPANY, OF DENVER, COLORADO

## METHOD OF FILMING COAL

No Drawing.

Application filed October 13, 1930. Serial No. 488,551.

This invention relates to a method and composition of matter for filming coal.

It is a well known fact that coal during transit and storage in yards, undergoes both physical and chemical changes, principally due to the absorption of oxygen from the air, commonly known as "weathering".

Among the detrimental effects of weathering are, a change in the coal size due to weakening of cleavages (the primary cause of excessive dust); loss of heating value; deterioration of burning quality and excessive absorption of moisture.

All of the above deteriorative effects of weathering on the coal are eliminated, by the use of the present invention, which briefly, consists in surrounding the freshly mined coal with a preserving film which is impervious to both air and water. The film after application must be impervious to air and water in order to eliminate the causes of weathering and thereby prevent the deteriorative effects stated hereinbefore.

Inasmuch as the preserving film excludes the air from contact with the coal, cleavage fracture due to weathering is prevented, and the formation of dust is practically impossible. The loss of heating value due to oxidation of the coal is prevented at the same time and the coal reaches the ultimate consumer with its heating value unimpaired. In fact the reduction of breakage and the prevention of oxygen absorption tends to increase the burning quality of the coal and the film itself adds to the heating value of the coal as will be more fully described herein-after.

Furthermore, the preserving film being impervious to water, prevents the absorption of moisture to an injurious extent, which obviously is of advantage in the storage, transit and ultimate use of the coal.

The film may be applied to the coal in any suitable manner, such as by passing the coal through a bath of the filming preparation in liquid form. It is essential that the filming preparation shall have all the preservative qualities hereinabove referred to and shall, at the same time, be inexpensive and easily applied, so that the filmed coal may be mar-

ked without material increase in the cost of production.

A filming composition well adapted for the purpose is composed of still residue obtained in the manufacture of benzol products in by-product coking plants, held in solution by the use of crude solvent. The still residue contains a large percentage of para coumarone in admixture with other resins and hydrocarbon oils and it is the film producing agent of the composition. The solvent serves as a carrier for the residue which in this manner, is readily applied to the coal.

A still residue used with satisfactory results consists of the tailings or residue above 180 degrees centigrade, obtained in refining benzol.

The crude solvent must be of a nature not deteriorative to the burning qualities of the coal and should, if possible, enhance the same.

Any oil may be used as a solvent, with or without agitation according to its nature. It is preferred, however, to employ as a solvent, benzol oil or its homologues.

In order to harden the film shortly after it has been applied to the coal, a suitable drier may be added to the solution. A drier which also acts as an oxidizing agent, is preferred since it promotes the burning qualities of the coal. Manganese dioxide is well adapted for the purpose, as it readily and quickly hardens the film on the coal, and as manganese dioxide at 500 degrees centigrade liberates oxygen available for efficient combustion.

In preparing the composition, the following proportions of its ingredients have been found to be productive of good results:

|                   |            |
|-------------------|------------|
| Still residue     | 5 gallons  |
| Crude solvent     | 45 gallons |
| Manganese dioxide | 1/4 pound  |

The film applied to the coal by the use of the solution is in appearance similar to a thin coating of lacquer and imparts to the coal the bright lustre of anthracite. The film, therefore, renders the coal easily distinguishable from other coals of similar kind, and in addition, greatly increases the heating value of the coal.

tion to its other qualities, may be said to perform the function of a trade-mark.

Another advantage of the preservation method, as stated hereinbefore, resides in an increase of the heating value of the filmed coal by reason of the fact that the preservative itself has a heating value of upwards of 18,000 B. t. u.

The film coating ignites readily and burns with a brilliant hot flame. At the same time, it tends to retain the coal gases until the surface temperature is raised to a point where efficient combustion is insured.

By virtue of the fact that the principal ingredient of the composition is a residue obtained in the operation of a by-product coking plant, which residue is of commercial value, and in view of the further fact that the material treated in the coking plant is the same as that to which the composition is applied, it will be apparent that coating the coal with the composition, does in no way, alter its characteristic properties or interfere with its uses for any purpose for which it is adapted in its original state.

It follows that the coated article is one which has a film composed of a substance which is of a nature identical or similar to that of the article itself, or, in the present instance, that the coal has a film composed of a coal product. This is a valuable and distinctive feature of the invention.

In brief, coal filmed by the above described method, is cleaner, of better appearance and of higher quality and is more economical in combustion than the same coal in its natural state.

It is to be understood that while the ingredients of the composition hereinabove described per se and in the given proportions, are at present preferred by reason of the good results obtained in their use, variations in both may be resorted to without departing from the spirit of the invention.

45 What I claim and desire to secure by Letters Patent is:

1. The method of filming coal comprising applying to the surface of the coal para coumarone in solution.

50 2. The method of filming coal comprising applying to the surface of the coal a still residue comprising substantially a large amount of para coumarone produced by refining by-products in coking plants, in solution.

55 3. The method of filming coal comprising applying to the surface of the coal a still residue comprising substantially a large amount of coumarone produced in refining benzol in solution.

60 4. The method of filming coal comprising applying to the surface of coal a water-insoluble, weatherproof material comprising substantially a large amount of para coumarone dissolved in benzol oil as a solvent.

65 5. The method of filming coal comprising

applying to the surface of coal a water-insoluble, weatherproof material comprising substantially a large amount of para coumarone dissolved in benzol oil as a solvent.

6. The method of filming coal comprising applying to the surface of coal a drying, water-insoluble, weatherproof material comprising substantially a large amount of para coumarone in an oil solvent.

7. The method of filming coal comprising applying to the surface of coal a water-insoluble, weatherproof material comprising substantially para coumarone, an oxidizing drier, and dissolved in oil.

8. The method of filming coal comprising applying to the surface of coal an oily, water-insoluble coal product, comprising substantially para coumarone, and subjecting same to a drying action to form a film.

9. The method of filming coal comprising applying to the surface of the coal para coumarone and manganese dioxide in solution.

10. The method of filming coal comprising substantially applying to the surface of the coal, a water-insoluble, weatherproof material containing para coumarone, benzol and manganese dioxide, and subjecting same to a drying action whereby to form a water-insoluble weatherproof film.

11. The method of filming coal comprising substantially applying to the surface of the coal, a water-insoluble, weatherproof material containing para coumarone, an oil solvent and manganese dioxide, and subjecting same to a drying action whereby to form a water-insoluble, weatherproof film.

12. The method of filming coal comprising substantially applying to the surface of the coal, a water-insoluble, weatherproof material containing para coumarone, benzol and a drying agent, and subjecting same to a drying action whereby to form a water-insoluble, weatherproof film.

13. The method of filming coal consisting in immersing the coal in a solution containing still residue having a large percentage of para coumarone, a solvent, and a drying agent, removing the coal from the solution and subjecting the coal to the oxidizing action of air to cause the adhering solution to dry and thereby form a protective film on the coal.

In testimony whereof I hereunto affix my signature.

KENNETH B. STUART.